

## UNITED STATES PATENT OFFICE

JOHN F. K. McCULLOUGH, OF DETROIT, MICHIGAN, AND BENJAMIN W. GILCHRIST, OF EAST ORANGE, NEW JERSEY, ASSIGNORS TO TERNSTEDT MANUFACTURING COMPANY, OF DETROIT, MICHIGAN, A CORPORATION OF MICHIGAN

## ELECTROPLATING BATH

No Drawing.

Application filed October 7, 1929. Serial No. 398,088.

This discovery relates to a new electro-plating bath and particularly to gold, silver, copper, brass, or bronze or zinc plating baths.

In plating with these metals, particularly 5 with copper for example, it has been the practice recently where large production of copper plating is used to use a double cyanide bath: that is, a bath made up of sodium cyanide and copper cyanide together with an 10 excess of free sodium cyanide. This sodium cyanide combines with the water of solution and the carbon-dioxide of the air to form sodium carbonate and at the same time there is liberated poisonous hydrocyanic acid gas. 15 The dissipation of the sodium cyanide also results in poor corrosion of the copper anode, poor conductance and very streaked deposits of copper.

In plating with brass and silver, the solutions 20 are at low temperature and the sodium cyanide does not attack the brass and the silver anodes as rapidly as is the case where the plating solution is warm or hot. With the zinc solution, which is ordinarily run 25 from 90° to 120° F., with the gold solution, which is run between 160° and 180° F. and the copper solution which is run at about 140° or 150° F. and sometimes as high as 180°, the destructiveness of the sodium cyanide and hence poor anode corrosion is quite 30 pronounced. Furthermore, in all these plating solutions, the free sodium cyanide is dissipated by reason of its reaction with the water of solution and the carbon-dioxide of 35 the air to form a hydrocyanic acid gas. This results not only in the liberation of poisonous gas but results in a deterioration of the conductivity of the bath. Also, it results in considerable expense as the sodium cyanide has 40 to be added two or three times a day, especially in the hot solutions. With the cool solutions, the sodium cyanide is added at much longer periods.

We have discovered that the excess sodium cyanide can be completely eliminated from 45 these double cyanide baths. In place of the excess sodium cyanide, we prepare a bath in which the sodium cyanide and the copper cyanide are exactly in the proportions at which 50 they combine to form a double cyanide.

With the other metal plating baths, this is substantially the practice but in all events, we take the double salts and eliminate the excess sodium cyanide. Other ingredients may or may not be present with these other baths. When we say the double salts, we mean that in each of these baths there is present the double salts of the metal and an alkali metal such as sodium cyanide or potassium cyanide. With the brass and bronze which are alloys, one takes the double salts of the two metals, to wit: sodium zinc cyanide and sodium copper cyanide; with bronze there is present, ordinarily, sodium copper cyanide and sodium zinc cyanide with considerably less zinc than is the case with the brass solution and the bath is run at a considerably higher temperature so as to plate out more of the copper.

In all these baths, we have found that in place of the excess sodium cyanide, we can use the Rochelle salts, to wit: sodium-potassium-tartrate. We find that in the copper solution it is desirable to add caustic soda. We find that with such a bath, especially when run, for instance, with copper, at 180° to 212° with a current of 4 to 6 volts very good anode corrosion, conductance and clear deposits of copper take place.

As an example of a copper bath, we use a solution that contains one ounce of copper cyanide to a gallon of water and a half ounce of sodium cyanide to a gallon of water and two ounces of caustic soda and three ounces of Rochelle salts. We give below a table 55 with a range of these ingredients which can be used with good results:

|         |       |      |                               |
|---------|-------|------|-------------------------------|
| 7.5-15  | g./l. | 1-2  | ozs. of copper cyanide        |
| 3.2-7.5 | g./l. | .5-1 | oz. of sodium cyanide         |
| 15-30   | g./l. | 2-4  | ozs. of caustic soda          |
| 22-120  | g./l. | 3    | saturation of Rochelle salts. |

Water—1 gallon

Temperature preferred 180°-212° F.

6-volt current

If, however, the proportions are not exact in starting, not a great deal of difficulty will be encountered as the heat will soon dissipate the excess sodium cyanide and in case of an excess copper cyanide, this would be taken up by the Rochelle salts to form a double tartrate of the copper and the alkali metal. This

will result in making the solution blue, from which no particular harm results. However, by adding more sodium cyanide, the double tartrate of the copper and the alkali can be 5 changed back into the double cyanide and the alkali tartrate.

It is not necessary to schedule the proportions in making up a bath of the other metal solutions as any chemist can figure out the 10 correct proportions of the ingredients that go to make up the double cyanide and substantially the same amount of Rochelle salts can be used as with the copper solution, although, experience will show that there can 15 be a variation of more or less of these salts. In the brass and bronze solution the caustic soda should be left out. It may or may not be used in the other solutions except that it is highly desirable with the copper solution. 20 In place of the Rochelle salts, one can substitute alkali citrate, such, for instance, as sodium or potassium citrate and also the alkali bitartrates such as potassium bitartrate may be used. Caustic potash may be used 25 instead of caustic soda. In the bronze, brass, and silver solutions, ammonium tartrate can be substituted for Rochelle salts.

We find that electro-plating baths made up 30 in this way result in deposits that are free from streaks and of good color, that the solution has better throwing power, can be operated with a greater range of temperature, without decomposition (100°-212° F.), can be operated with a greater range of current 35 density to say 10-100 amperes per square foot, and reduces the buffing cost. We estimate that the cost of this solution over a long run is only about 17% of the excess cyanide solution for the reason that we obviate the necessity of adding sodium cyanide.

We might add here that in these double solutions it is possible, of course, to use potassium cyanide but this is rather costly, and, of course, when the potassium cyanide 45 is used in the double cyanide, it is customary to use as the excess, potassium cyanide.

What we claim is:

1. An electroplating bath comprising a double cyanide of the metal to be deposited 50 and one of the two alkali metals, sodium and potassium, and a double salt made up of one of a group of organic compound ingredients which consists of the tartrates and citrates and one of the group of alkali metals, which 55 consists of potassium, sodium and ammonium, the proportions for the copper bath being 1 to 2 ounces of copper cyanide,  $\frac{1}{2}$  to 1 ounce of alkali metal cyanide and 2 to 4 60 ounces of caustic soda and 3 to 16 ounces of the double salts of the tartrate or citrate per gallon of water.

2. The bath claimed in claim 1 in which the temperature is approximately 180° F. to 65 212° F.

3. The bath claimed in claim 1 in which the voltage is approximately 6 volts.

In testimony whereof we affix our signatures.

JOHN F. K. McCULLOUGH. 70  
BENJAMIN W. GILCHRIST.

75

80

85

90

95

100

105

110

115

120

125

130